

## UNITED STATES PATENT OFFICE

2,330,111

## CASTING MAGNESIUM

William R. Caple, Evanston, Ill., and Richard I. Thrune, Midland, Mich., assignors to The Dow Chemical Company, Midland, Mich., a corporation of Michigan

No Drawing. Application August 1, 1942,  
Serial No. 453,248

7 Claims. (Cl. 22—188)

This invention relates to improvements in the casting of magnesium and magnesium-base alloys in temporary molds.

The production of commercially acceptable castings of magnesium and magnesium alloys presents a problem which is unique in foundry practice due to the affinity for both oxygen and nitrogen which this metal possesses, especially at elevated temperatures. In the molten state, at the temperatures employed in casting, the metal is capable of combining spontaneously with oxygen, which may be derived either from the air or from substances containing free or combined oxygen which are in contact with the metal, such as water, steam, or other compounds present in the material constituting the casting mold. This burning or oxidation of molten magnesium may at times be so violent as to approach explosiveness. Thus, it is practically impossible to make sound castings of magnesium in simple "green sand" molds, such as are used for casting other metals.

Because of this problem, it is conventional to incorporate in the material forming the mold some addition agent for overcoming the tendency of water or other oxygen compounds in the mold to attack magnesium when the latter is cast therein. For example, it has been suggested to mix sulphur or boric acid into a water-bound sand mold for casting magnesium to overcome harmful effects of air or water vapor on the metal. However, these substances have proved not to be wholly satisfactory, inasmuch as when a sufficient amount of either sulphur or boric acid is added to the molding sand to prevent oxidation of a casting of relatively heavy section, thin sections are liable to be pitted. On the other hand, if the amount of agent is reduced to a point where pitting of thin sections is minimized, heavier sections may be insufficiently protected from oxidation. Various other protective agents such as simple and complex fluorides have also been suggested for preventing the burning of magnesium when cast in water-bound molds, but these substances are likewise not altogether satisfactory, since they are lost rapidly during use and since they may cause the sand to swell, with resulting distortion of the mold. In addition, the use of fluorides is somewhat hazardous because of the toxicity of these materials.

In view of these difficulties, it is the principal object of the present invention to provide a method of casting magnesium and magnesium-base alloys in temporary molds in which there are utilized addition agents which effectively

protect the metal against oxidation during casting, but which are not subject to the disadvantages of agents heretofore known.

According to the invention, the tendency for oxidation or burning of magnesium and magnesium alloys when cast in temporary molds may be satisfactorily overcome by incorporating in the molding material prior to the casting of the magnesium a small proportion of an aromatic ester of a phosphorus acid. These new agents permit making castings of either relatively heavy or light section substantially without burning, pitting, or the formation of blow holes or similar flaws. They are less volatile under casting conditions than those heretofore used, so that their effectiveness is lost very slowly during repeated use of the sand. At the same time they do not have a detrimental effect on the molding quality of foundry sands, but actually render it workable for a longer period of time and lower the dry strength of the sand, making later shakeout much easier. In addition, the new agents and their thermal decomposition products are non-toxic and accordingly do not constitute a health hazard.

In so far as is known, any aromatic ester of a phosphorus acid may be employed as the addition agent of the invention. However, the aromatic tri-esters of phosphoric acid are preferred, especially the triaryl phosphates, such as triphenyl phosphate, tricresyl phosphate, di-phenyl-mono-orthoxenyl phosphate, tri-(para-tertiarybutyl phenyl) phosphate, di-(para-tertiary-butyl phenyl) monophenyl phosphate, di-orthoxenyl-mono-phenyl-phosphate, and (4-tertiary-butylphenyl) phenyl ortho-xenyl phosphate. However, other aromatic esters of phosphorus acids, such as the tri-haloaryl phosphates, e. g. tri-(2,4,6-tri-chlorophenyl) phosphate, aromatic tri-esters of phosphorous acid, e. g. di-(2-xenyl) phenyl phosphite, certain esters of thiophosphoric acid, such as phenyl di-(metatolyl) thiophosphate and di-phenyl ortho-xenyl thiophosphate, may also be used. Those esters which are liquid are ordinarily preferred because of their ease of application. Esters boiling at an absolute pressure of 5 millimeters of mercury in the range of 250° to 300° C. are most satisfactory, since they are sufficiently volatile to afford adequate protection to the magnesium without being so volatile as to be lost rapidly during use.

The amount of the new agent which may be employed varies with the size and type of casting to be made as well as with the nature of the mold-

ing material, which is usually foundry sand. In making large castings a greater proportion of the agent may be required than when relatively small castings are made. Normally, foundry molding material may be intimately mixed with from 0.5 to 10 per cent by weight of any one of the compounds previously mentioned, although usually about 1 to 5 per cent is satisfactory. Mixtures of two or more of these substances may be employed, the sum of which preferably does not exceed about 10 per cent. It is understood, however, that the quantity of one or more of such agents in any given case is a matter of judgment, governed more or less by the size and character of the casting.

In the casting of magnesium and its alloys according to the invention, the preparation of the mold and cores is carried out entirely in accordance with known practice, except that the phosphorus acid esters are used in place of the addition agents heretofore employed. In general, in the case of green-sand castings, the new agent is incorporated into the water-tempered foundry sand or synthetic sand, such as a silica-bentonite mixture, by mechanical mixing, after which the sand is formed into molds and cores, the latter with addition of a binder, in conventional manner. Alternatively, mold facings may be prepared from foundry sand mixed with the new agents, and the mixture applied to the pattern in the usual fashion. Again, the new agents may be dissolved in a volatile solvent, such as carbon tetrachloride, and the solution then sprayed on the mold parts which come in contact with the molten magnesium, or these parts may be dusted with a powdered solid triaryl phosphate.

The use of the new agents, furthermore, is not necessarily limited to molds made from sand, since other moldable materials such as graphite, pulverized carbon, or the like may be substituted for the sand. The agents are also useful in connection with semi-permanent molds, such as those made of plaster.

The following example will serve to illustrate the invention, but is not to be construed as limiting its scope.

#### Example

A water-tempered foundry sand having an A. F. A. permeability factor of about 80 was mulled together with 5 per cent by weight of di-(para-tertiary-butylphenyl) monophenyl phosphate, and the mixture was formed into a mold.

A casting was then prepared by pouring a quantity of Dowmetal H (a magnesium-base alloy containing 6.0 per cent aluminum, 3.0 per cent zinc and 0.2 per cent manganese, the balance being magnesium) into the mold, the pouring temperature being about 1400° F. The surface of the resulting casting was smooth, free from pits, blow holes, and oxidized areas.

Other modes of applying the principle of the invention may be employed instead of those explained, change being made as regards the details described, provided the method or mold recited in any of the following claims, or the equivalent thereof, be employed.

We claim:

15. 1. In a process of casting magnesium and magnesium-base alloys in temporary molds, the improvement which comprises incorporating an aromatic ester of a phosphorus acid into the mold material prior to the casting of the metal.
20. 2. In a process of casting magnesium and magnesium-base alloys in green-sand molds, the improvement which comprises incorporating between 0.5 and 10 per cent by weight of an aromatic tri-ester of phosphoric acid into the sand prior to the casting of the metal.
25. 3. A process according to claim 2 wherein the ester employed is a normally liquid tri-aryl phosphate.
30. 4. The method of casting magnesium and magnesium-base alloys in temporary molds which comprises incorporating into the molding material an aromatic ester of a phosphorus acid, forming a mold of the resulting mixture, and casting the metal therein.
35. 5. In a process of casting magnesium and magnesium-base alloys in sand molds, the method of minimizing oxidation of the metal during casting which comprises pouring the molten metal into a mold in which is incorporated, at least in the portions adjacent the molten metal, a small proportion of an aromatic tri-ester of phosphoric acid.
40. 6. A temporary mold for casting magnesium and magnesium-base alloys having mixed with the molding material a small proportion of an aromatic tri-ester of a phosphorus acid.
45. 7. A sand mold for casting magnesium and magnesium-base alloys having mixed with the sand between 0.5 and 10 per cent by weight of a triaryl phosphate.

WILLIAM R. CAPLE.  
RICHARD I. THRUNE.